

(No Model.)

G. L. HUXTABLE.

PROCESS OF MAKING PULP.

No. 269,291.

Patented Dec. 19, 1882.



Attest  
John S. Jones  
Eugene L. Brinkman.

Inventor  
George L. Huxtable,  
by Hood & Boyce,  
his Attorneys.

# UNITED STATES PATENT OFFICE.

GEORGE L. HUXTABLE, OF LAUREL, INDIANA, ASSIGNOR OF ONE-HALF TO  
SIMPSON & GAULT, OF CINCINNATI, OHIO.

## PROCESS OF MAKING PULP.

SPECIFICATION forming part of Letters Patent No. 269,291, dated December 19, 1882.

Application filed March 11, 1881. Renewed November 23, 1882. (No model.)

*To all whom it may concern:*

Be it known that I, GEORGE L. HUXTABLE, a citizen of the United States, residing at Laurel, in the county of Franklin and State 5 of Indiana, have invented certain new and useful Improvements in Processes of Making Pulp, of which the following is a specification.

My invention relates to an improvement in the process of reducing wood and other fibrous 10 articles to a pulp for paper-making.

The processes for reducing wood to pulp hitherto used were, first, by means of boiling the chips in a solution of caustic soda or other chemicals under steam-pressure. The cost of 15 the reduction by this process is very much more than by mine. Besides, I avoid the use of expensive machinery. Another process for reducing wood pulp by purely mechanical means is to take blocks of wood and hold them 20 against the face of coarse grindstones or emery-wheels. This process is objectionable, first, because of the large amount of power required and the slowness of the process; and, second, the pulp removed by the revolving stone is not 25 of uniform fineness, but requires regrinding, which in a great measure destroys the wood fiber and produces an inferior article of pulp.

My invention consists in reducing wood or other fibrous material to pulp by first reducing 30 the wood to small blocks by cutting or sawing, or by both cutting and sawing, until it is small enough to be fed into millstones in a manner similar to grain, except a continuous stream of water is introduced with the wood, which 35 is ground by the stones, and the water carries off the finer or pulpy parts as fast as it is reduced and prevents it from being retained long in the coarser mass, which would cut or injure the fiber. The product from the first set of 40 millstones is carried immediately into a second set, and the water in like manner carries off the finer portions as fast as reduced to prevent cutting or injury of the fiber, and this process of gradual reduction by regrinding it 45 in a finer set of mills is continued until the fiber is sufficiently reduced to form pulp.

My invention overcomes the objection existing in the ordinary mechanical processes of reducing wood pulp, and produces a superior 50 wood pulp by purely gradual mechanical reduc-

tion and at a much less cost than by older processes.

Other features of my invention will be fully set forth in the annexed description of the drawings.

In the accompanying drawings, Figure 1 represents a series of reducing-mills. Fig. 2 represents a sawing or cutting device.

A represents a series of saws, which are set close together, mounted upon an ordinary arbor or mandrel, B. These saws are preferably made of one-eighth of an inch or upward in thickness, with the teeth formed like ordinary crosscut buzz-saw, except the teeth are filed so that the edge is slightly beveled to incline 60 toward the log—that is, I use no set in the saw and file the teeth all upon one side, so that they will draw toward the log in cutting. The thickness of these saws is determined by the desired length of the fiber.

B' represents a log which is reduced to very coarse sawdust, somewhat resembling short splinters, of uniform length, and quite free from the dust or "flour of wood." Instead of using this kind of reducing-machine for the first step 75 of my process, a series of cutting-knives or a bark or bone grinding mill may be employed, the object being to reduce the wood to a fiber, and as free from dust as possible, to a sufficient fineness, so that it can be fed into a burr or 80 grinding mill.

Fig. 1 of the drawings shows a series of reducing-mills, C D E.

F G H represent common millstones, which preferably are sandstones. These stones are 85 dressed with furrows deeper at the eye and running out to a gradual or less depth toward the periphery, and the last or finishing set of stones, in which the furrow should terminate slightly within the peripheral line. It is desirable, also, to have the furrows nearer together than in the ordinary mills, as the grinding is done at the upper edge of the furrow. The more furrows the more rapid the operation. In practice I have usually used four sets of 95 these stones, but have sometimes used but three, as when one set of stones was being dressed the process was carried out by the remaining three sets and good results obtained.

I represents a water-pipe, which carries a 100

stream of water into the eye of the grinding-stone F.

K L represent spouts which are used to carry the water and fibers from one set of millstones 5 to the other, and they should have requisite pitch to accomplish this object.

M represents the hopper into which the fiber product prepared for grinding is fed into the stones. Care should be taken to adjust the 10 setting of these different stones so that the last set shall not be crowded in its work. In practice the work of gradual reduction is chiefly performed before the product passes to the last set of millstones, and by having a smooth 15 surface just at the periphery of the stones I am enabled to reduce any coarse particles that have escaped the proper reduction in the other sets of stones. This feature is not essential; but I deem it the preferable way of carrying 20 out the process. It is preferable to have each successive set of stones with the furrows shallower at the periphery than the preceding set. This is not absolutely essential; but it is essential to have the furrows decrease in depth as 25 they approach the periphery, and where they gradually terminate. In this respect they differ from ordinary grain-mills.

It is manifest that other fibrous material than wood may be reduced in the same manner, substantially, the different steps being somewhat varied.

The liquid pulp produced by my machine and process is prepared for use of paper or for commerce by a wet-mill in the ordinary way.

35 I claim—

1. The herein-described process of making pulp from wood or other fibrous material by the gradual reduction of said fiber by successive series of rubbings between a series of 40 grinding-mills constructed and arranged substantially as herein set forth.

2. The herein-described mode or process of the gradual reduction of wood or other fibrous material, which consists, first, in reducing the material to a coarse consistency suitable for 45 being fed into a grinding-mill, into which it is admitted with a stream of water to assist in rubbing, and thence carried into another set of millstones, where it is still further reduced, which gradual reduction by grinding-mills is 50 successively continued until the fiber is uniformly reduced to a finished pulp, substantially as herein set forth.

3. In the manufacture of pulp from wood or other fibrous material, a series of instruments 55 consisting essentially of a sawing or cutting mill, A, and a series of grinding-mills, C D E, or their equivalents, arranged in consecutive order, so that the product of the cutting-machine can be introduced into the first mill in 60 connection with a stream of water and pass through the series of mills, by which it is gradually reduced to a finished pulp, substantially as herein set forth.

4. A series of reducers, C D E, each consisting of a pair of mill grinding-stones the furrows of which are dressed to gradually terminate at or near the periphery, and adapted to a gradual reduction of wood or other fibrous material to a finished pulp by the successive 70 operation of the series, substantially as herein set forth.

In testimony whereof I have hereunto set my hand in the presence of two subscribing witnesses.

GEORGE L. HUXTABLE.

Witnesses:

J. H. CHARLES SMITH,  
JNO. E. JONES.